

United States Patent Office.

THOMAS SHAW, OF PHILADELPHIA, PENNSYLVANIA.

*Letters Patent No. 77,111, dated April 21, 1868*

IMPROVED MODE OF SURFACING SHEET-IRON AND METAL PLATES.

The Schedule referred to in these Letters Patent and making part of the same.

TO ALL WHOM IT MAY CONCERN:

Be it known that I, THOMAS SHAW, of the city and county of Philadelphia, Pennsylvania, have invented a new and improved Method of Surfacing Iron and Steel; and I hereby declare the following to be a full, clear, and exact description of the same, reference being had to the accompanying samples.

My invention consists in the application of carbon to the surface of iron or steel, during the process of hot-rolling, or other manipulation requiring heat.

The object is to prevent the rapid corrosion of iron in the air whilst heated, and to aid in producing a smooth surface on all wrought iron.

In order to enable others to use and practise my invention, I will proceed to describe its mode of operation.

The material applied to the iron consists of plumbago, animal fat, soda, and water, the valuable constituent of which is the plumbago.

The material can be applied to the heated surface of metal by dropping or rubbing it upon the rolls through which the metal has to pass; also by rubbing it upon the heated surface of the metal with a mop, adapted to the configuration of the iron.

It will be observed that carbon can be employed in combination with various other materials.

I therefore do not wish to confine myself to the materials in combination with the carbon, but

What I do claim, and desire to secure by Letters Patent, is—

The application of carbonaceous material to the heated surfaces of iron and steel, whilst being rolled or otherwise manipulated upon, substantially as and for the purpose set forth.

THOMAS SHAW. [L. S.]

Witnesses:

E. COBB,

ELIAS S. SHAW.